

## UNITED STATES PATENT OFFICE

2,668,159

## TEXTILE PRINTING WATER-IN-OIL EMULSIONS HAVING AS THE OIL PHASE A THERMOPLASTIC RESIN PLASTISOL EMULSIFIED IN A THERMOSETTING RESIN LACQUER

Edward F. Armatus, New York, N. Y., assignor to Sun Chemical Corporation, Long Island City, N. Y., a corporation of Delaware

No Drawing. Application January 4, 1951,  
Serial No. 204,492

7 Claims. (Cl. 260—29.4)

1

The present invention relates to coloring compositions for textile materials, and relates more particularly to pigmented emulsions especially adapted for imprinting textile fabrics.

The art of decorating and coloring textile fabrics by printing processes was formerly restricted almost completely to the use of various dyestuff materials. However, due to the high cost of many dyes, the involved and rather expensive processes required to imprint and fix the dyes upon the fabrics, the lack of clarity or sharpness of line in the finished print, and the deficiencies of many dyestuffs as regards light fastness, resistance to washing, etc., it was sought to employ the less costly and more light fast insoluble pigment materials as the coloring matter in coloring compositions suitable for imprinting textile fabrics.

However, the use of such coloring materials for textile printing presented many new problems not encountered in the use of dyestuffs. Since pigments, unlike dyestuffs, are insoluble materials and have no affinity for textile fabrics, it is necessary that these materials be employed in printing compositions which contain therein a material which has the ability to adhere to the fibers of textile fabrics and which, in the presence of pigment materials, acts so as to bind the pigment particles to the said fibers. It was therefore attempted to imprint fabrics with printing compositions containing pigment materials dispersed in a solution, in a suitable solvent therefor, of a film-forming resinous material, the solvent usually being of such character as to be readily removable from the imprinted fabric as by rapid evaporation thereof. Such coloring systems, however, were found to be unsuitable as printing compositions for textile materials since they adversely affected the character of the fabric by cementing the fibers together and, in many cases, by filling in the interstices between the fabric fibers with a solid film of binder and pigment, thereby imparting an undesirable stiffness and harshness of feel to the fabric. Further, prints made with such printing compositions were not too resistant towards the action of various dry cleaning fluids customarily employed in such cleaning operations.

The deficiencies present in the imprinted fabric occasioned by the use of such pigmented printing compositions as above described has been largely overcome by the use, as printing compositions for textile materials, of pigmented emulsions containing film-forming resinous materials as the binder component thereof, which resinous materials are

characterized by their ability to set to a solvent insoluble condition by a suitable thermal treatment. These compositions are usually made and employed in the form of water-in-oil or oil-in-

water emulsions, the oil phase generally comprising a pigmented solution or dispersion of a film forming thermosetting resinous material in solvents substantially immiscible with water. Since these compositions are applied to textile fabrics in the form of an emulsion, the resinous binder material which carries the pigment is deposited upon the fabric in the form of a discontinuous film, so that instead of completely covering the fabric structure with a continuous film of binder and pigment, only the individual fibers which make up the fabric structure are found to be coated with a film of binder and pigment. Upon application of such pigmented emulsions to textile fabrics by the conventional printing processes, and upon subsequent treatment of the imprinted fabrics at temperatures sufficient to effect setting of the resinous binder material upon the fabric to a solvent insoluble condition, a printed fabric is obtained which is lacking in the stiffness obtained by the use of pigmented resin solutions alone and which has a hand or feel to the touch substantially the same as the unprinted fabric.

However, fabrics printed or colored with such pigmented emulsions usually had one deficiency which caused serious concern among textile printers. This is the effect known as crocking, or the tendency of the color of the printed fabric to rub off onto other materials, such as other fabrics, when a sliding contact is made therebetween. As is evident, this is a highly objectionable characteristic in colored fabrics since in washing and cleaning operations, or even in ordinary use, such fabrics would tend to discolor other fabrics which came into contact therewith. Since such condition in the imprinted fabric tended to offset the advantages derived from the use of such pigmented emulsions as printing and coloring compositions for textile materials, it was desired to eliminate this condition as far as possible without sacrificing any of the other advantages obtained by the use thereof.

By this present invention there are provided pigmented emulsions especially adapted for imprinting and coloring textile materials by the conventional printing processes employed in the textile industry whereby crocking in the finished print is substantially eliminated. The use of the pigmented emulsions of the present invention in the printing of fabrics does not materially change

the hand of the fabric imprinted, nor does it cause any stiffening or excess weighting in the printed fabric. When the imprinted fabric is subjected to a subsequent thermal treatment as hereinafter set forth, the imprinted fabric is highly resistant toward fading or discoloration as, for example, by the loss of pigment due to the effect of washing or laundering operations thereon, or due to the effect which the solvents ordinarily employed in dry cleaning operations may have upon the fabric.

The textile printing compositions of the present invention are pigmented water-in-oil emulsions in which the continuous or oil phase comprises a lacquer, or a solution of a thermosetting resinous material in organic solvents, said solution having dispersed therein a plastisol of a synthetic thermoplastic resinous material, the organic solvents of the lacquer being substantially non-solvents for the resinous material of the plastisol.

The term "plastisol" as employed in the present invention refers to stable dispersions of a finely divided thermoplastic resinous material in which the entire dispersion medium consists of non-volatile liquid plasticizers. Plastisols may be prepared by mixing or milling a finely divided thermoplastic resinous material with a suitable plasticizer, the amount of plasticizer generally used being sufficient to wet the resin particles and to provide a relatively fluid mixture. Such mixing or milling may satisfactorily be carried out in a pony mixer or ball mill, care being taken to avoid undue heating of the mixture during such operations since excessive heating tends to cause fusion of the resinous particles of the dispersion. These dispersions can be converted into tough, flexible coatings and self-supporting films by utilizing any of the standard techniques for forming such coatings and films and by then treating the said dispersion at temperatures sufficient to effect fusion of the dispersed resin particles. Since the sole dispersion medium of plastisols are non-volatile liquid plasticizers which remain in the coating and films thus formed, the ratio of plastisol to resin in the original dispersion will, to a large extent, govern the character of the resultant film or coating. It has been found that in order to secure the particularly desirable results obtained with the textile printing compositions of the present invention, it is essential that the ratio of plasticizer to resin in the plastisols employed be within certain definite proportions as hereinafter set forth. The resins which have been found to be particularly useful in providing the textile printing compositions of the present invention when employed in the form of plastisols are the polymers of vinyl chloride and the copolymers of vinyl chloride and vinyl acetate.

The most satisfactory binder materials for utilization as the binder material of the oil phase of the emulsions of the present invention are the alcoholated melamine-formaldehyde thermosetting resinous condensates which comprise the reaction product of melamine, formaldehyde, and an alcohol, such as butyl alcohol or capryl alcohol, reacted to a point where the condensate is soluble in organic solvents or in mixtures thereof, such as a mixture of equal parts of mineral spirits and butyl alcohol. Also suitable for such use are alkyd-modified melamine-formaldehyde thermosetting resinous condensates, as for example, a melamine-formaldehyde resinous condensate

modified with a drying oil-modified glycerol-phthalate resin.

The solvent medium of the oil phase of the printing emulsions of the present invention may comprise any of the ordinary hydrocarbon solvents, both aliphatic and aromatic, and also any of the common terpene solvents, and usually comprises mixtures of these solvents together with certain of the lower aliphatic alcohols since the thermosetting resinous materials mentioned above are usually provided and employed as solutions of the resins in mixtures of either aliphatic or aromatic solvents with various alcohols, such as butanol or capryl alcohol.

The plasticizers employed in preparing the plastisols or resinous dispersions utilized in the printing compositions of the present invention are water-immiscible non-volatile liquid organic compounds which are ordinarily miscible with the common organic solvents and thinners employed in the emulsions of the present invention. Examples of such plasticizers include tricresyl phosphate, triphenyl phosphate, dibutyl phthalate, dioctyl phthalate, dibutyl sebacate and dioctyl sebacate. As has been pointed out hereinbefore, the ratio of plasticizer to resin in the plastisols employed in the printing compositions of the present invention should fall within certain definite proportions. For best results, the plastisols utilized in the present invention should have a ratio of plasticizer to resin within the range of from approximately 1 to approximately 2 parts by weight of plasticizer to approximately one part by weight of resin. The use of plasticizer in amounts substantially beyond the limits specified has an adverse effect upon the end results obtained in the finished product, too small an amount of plasticizer resulting in a rather stiff and brittle film of binder and pigment, and too large an amount of plasticizer providing a binder-pigment film which is too soft to prevent rub-off of the pigment particles from the imprinted fabric.

As pigment coloring material there may be utilized either dry colors, or dispersed colors; that is, colors wherein the pigment has been dispersed in a solvent suitable for use as a part of the solvent medium of the oil phase of the emulsion. In practicing the present invention, it has been found that the amount of pigment coloring material utilized in the compositions of the present invention should not exceed a ratio of approximately 1.5 parts by weight of pigment to one part by weight of combined resinous binder; that is, the combined weight of both the thermosetting resinous binder of the lacquer and that of the thermoplastic resinous material incorporated into the compositions of the present invention in the form of a plastisol. Further, the ratio of the thermoplastic resinous material of the plastisol to the thermosetting resinous binder of the lacquer portion of the oil phase of the printing compositions of the present invention should preferably be maintained within a range of from approximately one to approximately two parts by weight of the said thermoplastic resinous material to one part by weight of the said thermosetting resinous binder of the lacquer portion of the emulsions.

In providing compositions in accordance with the present invention, it has been found to be completely satisfactory and economical to furnish a concentrate which subsequently can be diluted prior to use to furnish a composition with the desired body for the particular operation by

which such materials are applied to the fabric. In operations where a concentrate is furnished the user may dilute such concentrate with a suitable colorless emulsion, until a composition of the necessary flow properties and containing the amount of coloring material necessary for a particular printing operation has been obtained. Thereafter such printing may be effected by utilization of the equipment ordinarily employed in textile printing operations. When printing is completed, the colored fabric then is treated at elevated temperatures of the order of 300-350° F. for approximately one minute to effect removal of the volatile material present and to complete the setting of the coloring material upon the fabric.

A colorless water-in-oil emulsion (clear), suitable for diluting the pigment concentrate of the present invention, is provided as follows. A clear concentrate is prepared by emulsifying, as by stirring under high speed agitation conditions, the following material in the proportions set forth.

*Example 1*

|                                                                                       | Parts by weight | 25 |
|---------------------------------------------------------------------------------------|-----------------|----|
| Drying oil-modified glycerol-phthalate resin<br>(40% resin solids in mineral spirits) | 70              |    |
| Xylol                                                                                 | 5               |    |
| Ammonium sulfate                                                                      | 10              |    |
| Dialyzed waste sulfite liquor of U. S. P.<br>No. 2,201,812                            | 10              |    |
| Water                                                                                 | 5               |    |
|                                                                                       | 100             |    |

The clear concentrate provided as in Example 1 is then diluted and emulsified with Varsol and water in the proportions set forth in Example 2 to provide a water-in-oil emulsion suitable for diluting the pigment concentrate hereinafter set forth to the degree of printing consistency and shade of color desired.

*Example 2*

|                                | Parts by weight | 25 |
|--------------------------------|-----------------|----|
| Clear concentrate of Example 1 | 2.5             |    |
| Varsol                         | 22.5            |    |
| Water                          | 75.0            |    |
|                                | 100.0           |    |

The pigment concentrates of the present invention are water-in-oil emulsions in which the aqueous phase consists essentially of water and in which the oil phase comprises a lacquer comprising a solution of a thermosetting resinous binder material in substantially water-immiscible organic solvents, the said lacquer having dispersed therein a plastisol of a synthetic thermoplastic resinous material. As mentioned hereinbefore, plastiols are stable dispersions of a finely divided thermoplastic resinous material in which the entire dispersion medium consists of non-volatile liquid plasticizers. Therefore, the plasticizers and the vinyl resins of the following illustrative examples of the pigment concentrates are firstly combined into plastisol form and then admixed with the remaining materials which constitute the pigment concentrates and the whole is then emulsified by suitable means as, for example, by high speed agitation. The organic solvents utilized as the solvent medium of the oil-phase of the present emulsions are substantially non-solvents for the thermoplastic materials of the plastiols employed in the present invention. However, the same solvents act as diluents for the plastiols. The plasticizer

component of the plastiols acts so as to wet the resinous material thereof, constitutes the dispersant thereof, and as such forms a strong attachment for the dispersed resin particles. It is believed that when the plastiols are admixed with the remaining constituents which make up the emulsions of the present invention, the plastiols become thoroughly dispersed and suspended in the lacquer portion of the emulsions with the plasticizer portion of the plastiols acting as the suspension medium for the finely divided, dispersed thermoplastic resinous particles.

Illustrative examples of the pigment concentrates of the present invention are given below. In preparing such concentrates, satisfactorily all of the material may be charged to a high speed mixer and agitated until the requisite dispersion and emulsification is completed. To obtain the required degree of dispersion when a dry color is employed as the coloring material of the emulsion, the mixture should be passed through a roller mill or preferably be admixed and milled in a ball mill or pebble mill.

*Example 3*

|                                                                                                          | Parts by weight | 25 |
|----------------------------------------------------------------------------------------------------------|-----------------|----|
| Plastiols:                                                                                               |                 |    |
| Polyvinyl chloride                                                                                       | 8.0             |    |
| Tricresyl phosphate                                                                                      | 15.0            |    |
| Butylated melamine-formaldehyde resinous condensate (50% resin solids in 25 mineral spirits, 25 butanol) | 6.0             |    |
| Amyl alcohol                                                                                             | 12.0            |    |
| Turpentine                                                                                               | 42.0            |    |
| Phthalocyanine blue pigment                                                                              | 11.0            |    |
| Water                                                                                                    | 6.0             |    |
|                                                                                                          | 100.0           |    |

*Example 4*

|                                                                                                          | Parts by weight | 25 |
|----------------------------------------------------------------------------------------------------------|-----------------|----|
| Plastiols:                                                                                               |                 |    |
| Polyvinyl chloride                                                                                       | 10.0            |    |
| Diocetyl phthalate                                                                                       | 10.0            |    |
| Butylated melamine-formaldehyde resinous condensate (50% resin solids in 25 mineral spirits, 25 butanol) | 6.0             |    |
| Amyl alcohol                                                                                             | 10.0            |    |
| Turpentine                                                                                               | 45.0            |    |
| Phthalocyanine blue pigment                                                                              | 12.0            |    |
| Water                                                                                                    | 7.0             |    |
|                                                                                                          | 100.0           |    |

*Example 5*

|                                                                                                          | Parts by weight | 25 |
|----------------------------------------------------------------------------------------------------------|-----------------|----|
| Plastiols:                                                                                               |                 |    |
| Copolymer of vinyl chloride and vinyl acetate containing approx. 5% vinyl acetate                        | 5.0             |    |
| Diocetyl phthalate                                                                                       | 5.0             |    |
| Butylated melamine-formaldehyde resinous condensate (50% resin solids in 25 mineral spirits, 25 butanol) | 15.0            |    |
| Amyl alcohol                                                                                             | 10.0            |    |
| Turpentine                                                                                               | 43.0            |    |
| Phthalocyanine green pigment                                                                             | 12.0            |    |
| Water                                                                                                    | 10.0            |    |
|                                                                                                          | 100.0           |    |

Following the procedure hereinbefore outlined, the pigment concentrates of the above illustrative examples provide water-in-oil emulsions containing a continuous oil phase having suspended therein a dispersion of a finely divided thermoplastic resinous material and plasticizer. These emulsions may be diluted to any degree

desirable with the clear emulsion of Example 2 to provide the printing compositions of the present invention.

By the use of plastisols of the thermoplastic resinous material herein set forth as part of the oil phase of the pigmented emulsions of the present invention, there are provided printing compositions for textile materials whereby crocking in the finished print is substantially eliminated. Apparently the use of such materials in the form employed in the compositions of the present invention in some manner improves the pigment binding properties of these emulsion systems. Just why the plastisol dispersion should have such effect upon the finished print may possibly be explained by the fact that since the resinous material of the plastisol is present in the printing composition as a suspension of finely divided resin particles in the oil phase thereof, upon application of the said printing compositions to textile fabrics as by the conventional printing processes, the thermoplastic resinous material is deposited upon the fabric in the form of finely divided discrete particles interspersed throughout the pigmented thermosetting resinous film. It may be that upon subsequent heat treatment of the imprinted film, the plasticizer present in the imprinted film acts as a flux whereby the dispersed thermoplastic resin softens and flows together to form a protective film over or about the pigment particles and the thermosetting resinous binder materials which bind the pigment particles to the fabric. However, such explanation is merely theoretical and is not to be construed as a teaching of the actual manner in which the improved pigment binding properties are secured with the compositions of the present invention.

While the above products and processes constitute preferred embodiments of the present invention, changes may be made therein without departing from the scope of the present invention as defined in the appended claims.

What is claimed is:

1. A coloring composition for textile materials comprising pigment dispersed in an emulsion containing a discontinuous phase consisting essentially of water, and a continuous oil phase comprising a dispersion in a non-volatile liquid plasticizer of a thermoplastic resinous material selected from the group consisting of a homopolymer of vinyl chloride and a copolymer of vinyl chloride and vinyl acetate, said dispersion being suspended in a lacquer comprising a thermosetting resinous binder selected from the group consisting of alcoholated melamine-formaldehyde resinous condensates and alkyd-modified melamine-formaldehyde resinous condensates in organic solvents which solvents are substantially non-solvents for said dispersed thermoplastic resinous materials, the ratio of plasticizer to said thermoplastic resinous material being within the range of from approximately one to approximately two parts by weight of plasticizer to one part by weight of said resinous material.

2. A coloring composition for textile materials comprising pigment dispersed in an emulsion containing a discontinuous phase consisting essentially of water, and a continuous oil phase comprising a dispersion in a non-volatile liquid plasticizer of a homopolymer of vinyl chloride, said dispersion being suspended in a lacquer comprising a thermosetting resinous binder selected from the group consisting of alcoholated mel-

amine-formaldehyde resinous condensates and alkyd-modified melamine-formaldehyde resinous condensates in organic solvents which solvents are substantially non-solvents for said dispersed

5 polymer of vinyl chloride, the ratio of plasticizer to said polymer of vinyl chloride being within the range of from approximately one to approximately two parts by weight of plasticizer to one part by weight of said polymer of vinyl chloride.

10 3. A coloring composition for textile material comprising pigment dispersed in an emulsion containing a discontinuous phase consisting essentially of water, and a continuous oil phase comprising a dispersion in a non-volatile liquid

15 plasticizer of a copolymer of vinyl chloride and vinyl acetate, said dispersion being suspended in a lacquer comprising a thermosetting resinous binder selected from the group consisting of al-

20 coholated melamine-formaldehyde resinous condensates and alkyd-modified melamine-formal-

25 dehyde resinous condensates in organic solvents which solvents are substantially non-solvents for said dispersed copolymer of vinyl chloride and vinyl acetate, the ratio of plasticizer to said co-

30 polymer of vinyl chloride and vinyl acetate being

within the range of from approximately one to approximately two parts by weight of plasticizer to one part by weight of said copolymer of vinyl

chloride and vinyl acetate.

35 4. A coloring composition for textile materials according to claim 1 in which the plasticizer is dioctyl phthalate.

5. A coloring composition for textile materials according to claim 1 in which the plasticizer is tricresyl phosphate.

35 6. A coloring composition for textile materials comprising pigment dispersed in an emulsion containing a discontinuous phase consisting essentially of water, and a continuous phase comprising a dispersion in a non-volatile liquid plasticizer of a thermoplastic resinous material selected from the group consisting of a homo-

40 polymer of vinyl chloride and a copolymer of vinyl chloride and vinyl acetate, said dispersion being suspended in a lacquer comprising a butylated melamine-formaldehyde resinous condensate in a solvent mixture comprising mineral

45 spirits and butanol, the ratio of plasticizer to said thermoplastic resinous material being within the range of from approximately 1 to approximately 2 parts by weight of plasticizer to one part by weight of said resinous material.

50 7. A coloring composition for textile materials comprising pigment dispersed in an emulsion containing a discontinuous phase consisting essentially of water, and a continuous phase comprising a dispersion in a non-volatile liquid plasticizer of a copolymer of vinyl chloride and vinyl acetate, said dispersion being suspended in a lacquer comprising a butylated melamine-form-

55 aldehyde resinous condensate in a solvent mixture comprising mineral spirits and butanol, the ratio of plasticizer to said copolymer of vinyl chloride and vinyl acetate being within the range of from approximately 1 to approximately 2 parts by weight of plasticizer to one part by weight of

60 said copolymer of vinyl chloride and vinyl acetate.

65 EDWARD F. ARMATYS.

70 References Cited in the file of this patent

UNITED STATES PATENTS

| Number    | Name          | Date          |
|-----------|---------------|---------------|
| 2,374,602 | Kienle        | Apr. 24, 1945 |
| 2,431,078 | Powell et al. | Nov. 18, 1947 |
| 2,558,053 | Lee           | June 26, 1951 |